

# UNITED STATES PATENT OFFICE.

GEORGE H. PENDLETON, OF BUSCH, OKLAHOMA.

## PROCESS OF TANNING.

No. 876,583.

Specification of Letters Patent.

Patented Jan. 14, 1908.

Application filed June 25, 1907. Serial No. 380,785.

To all whom it may concern:

Be it known that I, GEORGE H. PENDLETON, a citizen of the United States, residing at Busch, in the county of Roger Mills and State of Oklahoma, have invented a new and useful Process of Tanning, of which the following is a specification.

The principal object is to provide a novel, cheap and thoroughly effective method or process of tanning hides, pelts or the like.

In carrying out the invention, if the hides or pelts are not soft, they are soaked in clear water until they become perfectly pliable. They are then placed on a beam and all the loose flesh is removed after which they are thoroughly washed in warm soapsuds. The hides or pelts are thus prepared for the solution for removing the hair or for tanning with the hair on. If the hair is to be removed, the pelt is placed in strong lime water for two or three hours until the hair slips easily. It is then washed in clear water, and the hair is removed in the well known manner, care being of course taken not to break the grain of the hide. The lime is then soaked or washed out thoroughly.

In certain portions of the country where the water is impregnated with gypsum, to four gallons of water is added one-fourth of an ounce of sodium carbonate and one-fourth of an ounce of ammonia. These ingredients are boiled together for five minutes and serve to act upon the gypsum in such a manner that it will have no deleterious effect on the hereinafter described tanning bath and process. Where pure water is obtainable, the above step is of course not necessary. Afterwards two pounds of gum gambier, placed in a small sack of thin muslin, is introduced thereinto and is boiled therewith until a pure reddish color is obtained. The bath is thereupon allowed to cool to a temperature that will not burn the hides or pelts, and said hides or pelts are then introduced, sufficient bath being employed to cover the same. They are allowed to remain in this bath from six to twenty-four hours, according to their size, and the pelt is then scraped off in the usual manner. After the hides or pelts have been thus subjected to this preliminary bath, one-fourth ounce of gum arabic one-fourth ounce of oil of hops and one-fourth ounce of fluid extract of wild cherry bark of the character described in the *U. S. Pharmacopœia* are stirred well into the above described

bath. The hides are then placed in this final bath, and are allowed to remain until thoroughly tanned which will take from three to fifteen days according to the thickness of the hide. Finally upon the removal of the hides or pelts, they are oiled with fish oil on both sides. The result is excellent leather that can be employed for any well known purpose.

There are a number of advantages for the method above described. In the first place, no machinery is necessary for smoothing the leather after the same has been tanned, for in the present process the soda and the mixture of the extract of wild cherry bark, oil of hops and gum arabic, makes the leather slick and smooth without the use of rollers. The hides are carefully prepared. The ammonia eliminates all greases from the skins, and the soda and gum gambier together produce an excellent color, besides preserving the grain of the leather and causing the pelts to relax so that the pores are open. The final bath enters these pores and constitutes an excellent preservative for the fibers of the leather. Moreover the ingredients employed are not of an acid nature, and will not burn or otherwise injure the hides while tanning the same.

Having thus fully described my invention, what I claim as new, and desire to secure by Letters Patent, is:—

1. The process of tanning hides, pelts, and the like, which consists in first introducing the hide or pelt into a bath containing a tanning and coloring material, allowing it to remain therein for a period of time, afterwards adding gum arabic, oil of hops and extract of cherry to said bath, and allowing the hide or pelt to remain in the final compound until tanned.

2. The process of tanning hides, pelts, and the like, which consists in softening the hide or pelt, introducing the same into a bath consisting of water, an alkali, ammonia, and a coloring and tanning material, allowing it to remain therein, then adding to the bath gum arabic, oil of hops and extract of wild cherry, and allowing said hide or pelt to remain therein until tanned.

3. The process of tanning hides, pelts, and the like, which consists in first softening the hide or pelt and removing the flesh therefrom, preparing a preliminary bath by boiling together water, soda and ammonia, afterwards adding gum gambier and boiling the same,

allowing the bath to cool, placing the hides or pelts therein for a predetermined period, adding to said bath, gumi arabic, oil of hops and extract of wild cherry, allowing the hide or pelt to remain until tanned, removing the hide or pelt from the final bath, and oiling said hide or pelt.

In testimony, that I claim the foregoing as my own, I have hereto affixed my signature in the presence of two witnesses.

GEORGE H. PENDLETON.

Witnesses:

A. B. WISDOM,  
O. H. CAFKY.